

## UNITED STATES PATENT OFFICE

2,171,744

## CAST METALLIC DENTURE

Cornell Joel Grossman, Millburn, N. J.

No Drawing. Application May 23, 1939,  
Serial No. 275,230

3 Claims. (Cl. 75—171)

This invention relates to metallurgy and more particularly to an alloy suitable for use in the manufacture of cast dentures and the like.

In the manufacture of metallic dentures the 5 alloy composition employed must be stainless and non-corrosive towards various acid and alkaline re-agents present in the mouth of various foods and liquids. The alloy also must be wear-resistant and the alloy must be variable as to percentages of the several constituents to a sufficient extent and flexibility permitting its use under a wide variety of service conditions. Moreover the alloy composition must be adapted to be readily cast free from blow-holes and with a minimum 10 of material surplus, by the ordinary methods practised in the art.

The present invention aims to provide an alloy adapted to meet these many conditions and further aims to provide a denture comprised of the 20 said alloy. The alloy composition of the present invention comprises a base consisting of cobalt and chromium in such relative proportions of the cobalt to give the required strength, toughness and where resistant properties are desired, and 25 chromium in sufficient amount to render the base stainless and corrosion-resistant. Into this base I may incorporate manganese or silicon or both in such amounts as will be necessary to completely deoxidize the alloy and to completely neutralize the deleterious effect of any sulphur or carbon present in the base and I may also incorporate a percentage of molybdenum or tungsten or both in such an amount as will augment the 30 normal strength and rigidity of the base. Into 35 the base or base improved by additions of one or more of the metals manganese, molybdenum and tungsten, I incorporate a sufficient percentage of boron as will effectively protect the alloy constituents from oxidation during the subsequent 40 re-melting and casting to form dentures. In the manufacture of dentures it is customary in the art to melt the alloy in an open crucible by impinging thereon the open flame of oxyacetylene, or oxy-hydrogen blow torch. When fully molten 45 the alloy is centrifugally cast into a mold wherein relatively rapid solidification occurs. Heretofore in the art it has been difficult to manufacture cast dentures of metals in this manner due to the fact that it is impractical to employ a protective slag over the metal during the melting and casting operations, as the slag, when used, also entered the mold and was entrapped by the rapidity of solidifying metal, causing blow-holes, voids and the like. When however a protective 50 slag was not used during the melting operation of

chromium containing alloys, excessive oxidation of the metal constituents occurred and voids caused by oxide and gas occlusions are obtained. This circumstance has greatly limited the use and adaptation of chromium-containing alloys, particularly in the forming of cast dentures, due to the fact that when molten or during melting the chromium contents of such an alloy or alloys rapidly oxidize to form difficultly fusible oxide compounds even though the alloy has been covered or protected by readily fusible slag materials. 5

I have found that the most effective way to prevent the oxidation of the chromium in chromium containing alloys is to incorporate in the 10 alloy an alloy-constituent which is more readily oxidisable than the chromium and which on oxidation forms a relatively low melting slag operating to protect the alloy from direct contact with oxidizing agents. Boron is the only alloy 15 constituent of which I am aware that will accomplish this desired result. 20

The amount of boron I may incorporate in the alloy composition of the present invention may vary widely without departure. I have successfully employed as low as 1.00% and as high as 25 10%. Under very expert manipulating conditions of melting and casting a boron content of less than 1.0% probably can be employed but under the ordinary manipulating conditions of melting and casting I prefer to have present in 30 my alloy about 5.0% boron, as this amount permits of repeated re-melting without detrimental results to the alloy. The excess boron does not appear to be deleterious in the alloy but to the contrary appears to increase the fluidity of the 35 alloy when molten and the ease with which it may be cast, and cast dentures of my alloy containing 5.0% or more of boron appear to be more sharply defined than those containing 1 to 2% boron. This amount of boron, moreover, appears 40 to beneficially affect the physical properties of the alloy, making it of finer grain structure and improving its hardness and luster.

In my alloy composition I prefer to limit any 45 iron content to less than 1.00%. Iron in amounts greater than this, while being of advantage in some respects, such as giving added strength and ductility, detrimentally affect the corrosion resistance properties and require added chromium to counteract the same. For this reason I prefer to limit my invention to a cobalt chromium base with iron less than 1.0%. In this base alloy the chromium content may vary from 5% to 45% and the cobalt content may vary from 45% to 55% with the remainder of the alloy consisting of 55

- boron up to 10% but preferably about 5% and manganese 1 to 2%, or silicon up to 1% or both. I find it preferable to increase the cobalt with decrease in chromium within the ranges specified 5 although this relation is not empirical but solely for the purpose of maintaining relatively constant corrosion resistance properties in the alloy. Where molybdenum or tungsten or both are added to the alloy as stiffening constituents, I 10 prefer to add these elements as replacements for part of the cobalt and in this respect the cobalt, molybdenum and tungsten are to be considered to be substantial equivalents, although each in addition contribute to the corrosion resistant 15 properties of the alloy. The molybdenum content may be as high as 8% but preferably should be in the range 2 to 4%. The tungsten content may be as high as 4%, but preferably should be in range of 1 to 2%.
- 20 As an example of the present invention, alloys that I have found most suitable for general purpose used in the casting of dentures have the following analyses:

| 25             | I                | II      | III             |
|----------------|------------------|---------|-----------------|
|                | Percent          | Percent | Percent         |
| Chromium.....  | 12 $\frac{1}{2}$ | 25      | 7 $\frac{1}{2}$ |
| Titanium.....  | 12 $\frac{1}{2}$ | 5       | 7 $\frac{1}{2}$ |
| 30 Cobalt..... | 60               | 62      | 80              |
| Boron.....     | 5                | 5       | 5               |
| Manganese..... | 1                | 1       | 0               |
| Iron.....      | 0                | 1 max.  | 0               |
| Silicon.....   | 0                | 1       | 0               |

35 Alloys suitable for the same purpose but stronger and more suitable for bridge-work are similar to composition No. 1, but contain molybdenum 2-8% with the cobalt reduced a corresponding amount or tungsten 1-4% with the cobalt reduced to a corresponding amount.

40 Where a softer alloy is desired, as in forming of pins, bars and the like, which subsequently are to be bent in shape, I increase the cobalt content to about 90% and lower the chromium contents to less than 10% with about 1% of 45 boron or manganese or 1% of both manganese and boron. The boron content of this alloy operates to facilitate the subsequent weld attachment of these pins, or bars, or clasps to a cast denture and even permits the casting of the denture directly unto the pin or clasp as heretofore practised in the art with other metals.

50 In the manufacture of the alloy composition of the present invention I sometimes prefer a chromium titanium alloy instead of chromium as an ingredient and a manganese boron alloy. These alloys should be preferably substantially free from carbon and from iron. I then mix the

chromium, titanium and manganese boron alloys together with cobalt, preferably in small-sized pieces, in such relative amounts as will give me the alloy composition desired, and melt the same down in the electric induction furnace under 5 conditions protecting the metal from oxidation. When fully molten the alloy is cast in the mold adapted to form relatively small diameter rods which after solidification may be cut or broken into relatively small pieces.

10 In the forming of dentures of this alloy, a sufficient amount of these small-sized pieces of rod is placed in an open crucible and is melted by the direct application thereon of the oxyacetylene or oxy-hydrogen flame and as soon as the 15 metal becomes molten and fluid the molten metal is cast centrifugally into the denture mold as heretofore practised in the art. The thus formed cast denture will be substantially free from blow-holes, voids or oxide and slag inclusions. Any 20 boron which is oxidized during the melting prior to casting, forms such a fluid slag that on entering the mold during casting the same does not interfere with the entrance of the molten metal into the finest crevices of the mold, and a clearly 25 defined sound casting will be obtained.

Satisfactory dentures may be cast from an alloy of 3% to 10% of chromium; 3% to 10% titanium; 1 to 10% boron, balance cobalt.

For greater rigidity the chromium is increased 30 and excellent dentures are obtainable from a casting alloy comprising 3-45% chromium; 1-10% boron; .2-.2% silicon; .2-.5% manganese; .2-.20% titanium; balance cobalt. The titanium and chromium can be added as a titanium chromium 35 alloy. The boron content may be increased without deleterious effect.

40 From the above description of the present invention, it will be apparent that the same may be widely varied as to alloy composition without departure from the invention and all such modifications and variations are contemplated as may fall within the scope of the following 45 claims.

What I claim is:

1. An alloy suitable for use in the manufacture of substantially sound non-oxidized castings and the like, said denture consisting of 3-10% chromium; 3-10% titanium; 1-10% boron, balance cobalt.
2. A casting alloy for denture and the like, comprising 3-45% chromium; 1-10% boron; 1-30% titanium, balance cobalt.
3. A casting alloy for denture and the like, comprising 5-15% boron; 1-30% titanium; 3-45% chromium; balance cobalt.

CORNELL JOEL GROSSMAN.